

## UNITED STATES PATENT OFFICE

ADOLF BECK, WALTHER SCHMIDT, AND GUSTAV SCHREIBER, OF BITTERFELD, GERMANY, ASSIGNORS TO I. G. FARBENINDUSTRIE AKTIENGESELLSCHAFT, OF FRANKFORT-ON-THE-MAIN, GERMANY, A CORPORATION OF GERMANY

## METHOD OF TREATING MOLTEN MAGNESIUM AND ITS HIGH-PERCENTAGE ALLOYS

Application filed August 20, 1928, Serial No. 300,840, and in Germany March 4, 1927.

This invention relates to the treatment of magnesium and its high-percentage alloys in the molten state.

It is well known that the air-exposed surfaces of molten easily oxidizable metals such as magnesium and its high-percentage alloys readily form films of a generally exceedingly tenuous though sometimes decidedly tough structure by reaction with the atmosphere. 5  
5 It is hardly possible to determine the composition of these films accurately; it may be supposed that they chiefly consist of oxide and nitride compounds of the various constituents of the alloys, though we do not wish 10 to limit ourselves by this explanation, the expression "reaction" covering effects produced by chemical as well as physical processes. These films are also formed whenever a free 15 jet of molten metal is exposed to the atmosphere, for instance, in pouring the metal from ladles or melting pots into molds. Although 20 these layers are in such cases hardly visible, they are notwithstanding of noticeable influence in foundry practice since they are apt to 25 tear up during the casting operation, the bits of the layer are swept into the mold, and every particle of these films occluded by the casting interrupts the continuity of its inter-crystalline structure thus impairing the 30 soundness of the product. Another difficulty arises from the fact that particles of fluxes or other foreign substances floating on the 35 surface of the molten metal in the pot, frequently adhere to these films and are thus also frequently swept into the moulds forming inclusions in the castings of a decidedly undesirable nature.

The present invention is based on the observation that, during the pouring operation, 40 this film also rapidly forms on every surface of the metal coming into contact with air. This applies not only to the surface of the casting pool, but more particularly also to the jet of flowing metal. We have discovered 45 that by a particular method of pouring the metal, this film, once it is formed, can be held in a stationary position, forming a kind of hose through which the metal flows as though through a pipe. The reaction products constituting the hose are thus efficiently

prevented from entering the mold as long as the hose is kept intact, and at the same time the flowing metal itself is protected from further oxidation by the hose which is practically impermeable to the reactive constituents of the air. Thus a continuous coherent film is formed covering the surface of the metal in the pot as well as the jet of flowing metal and the metal in the casting pool.

This film being of a decidedly tenuous though to a certain degree also tough structure considerable care is required to prevent it being severed, the latter resulting immediately in it being drawn into the casting. The preservation of the continuous structure of the film depends largely on the rate of the flow of metal when being poured from the pot. As a rule the rate of flow is regulated by tipping the ladle or crucible, by which procedure the mouth of the pot is lowered or raised simultaneously. Any sudden movement, however, particularly a raising, of the pot should carefully be avoided, because the protective film becomes easily overstressed and is then severed and its pieces swept into the mould. It is rather preferable to effect the tipping of the crucible by using its mouth as a pivot point so as to keep a fixed distance between the mould and the mouth of the pot during the whole pouring procedure. By this means it is possible to prevent the film from being severed and moving along with the metal into the mould. Particles of fluxes or slag floating on the surface of the metal in the pot are embedded in this film and therefore cannot be swept into the mould as long as the film of reaction products remains in its position on the surface of the metal.

When the mould is filled completely the crucible is taken away, thus separating it from the hose which now falls down on the casting pool without affecting the casting itself.

The annexed drawing gives a diagrammatic view of the conditions prevailing during the casting operation according to our invention. The crucible which it will be noticed is tipped, with the mouth being the pivot point is reproduced in two positions cor- 95 100

responding to the preliminary (1) and final (1') stages of the pouring procedure. 2 is the sand mould with the casting 3 and with the casting pool 5 filled with metal, while 4 delineates the film of reaction products (for the sake of clearness reproduced far thicker than is in reality the case) resting upon the casting pool 5, suspended by the mouth of the crucible and extending right over the surface of the metal in the pot.

10 The stability of the hose may be furthermore favourably influenced by adding to the atmosphere surrounding the flowing metal and the molten metal in the ladle or crucible substances capable of forming reaction products with the metal suitable to reinforce the structure of the film forming the hose. To this effect we prefer to spray finely divided sulphur over the jet of metal during the pouring operation.

15 The number and the shape of the gates of the mould is to be calculated in accordance with the above-described method; to this end it will often be necessary, in the case of 25 larger castings, to cast from several small crucibles instead from a large one, if when using the latter the conditions for preserving the hose cannot be fulfilled.

We claim:

30 1. A method of protecting a jet of molten magnesium and high-percentage magnesium alloys from oxidation, comprising the step of keeping the point of issue of the metal from the pouring vessel in a substantially 35 fixed position relative to the gate of the receiving mold whereby the jet of metal between the pouring vessel and the receiving mold in contact with the air forms a rigid hose through which the remainder of the 40 metal in the pouring vessel can flow without contact with the air.

45 2. A method of protecting a jet of molten magnesium and high-percentage magnesium alloys from oxidation, comprising the step of keeping the point of issue of the metal from the pouring vessel in a substantially 50 fixed position relative to the gate of the receiving mold, and maintaining a substantially constant rate of flow of the metal by steadily 55 tilting the pouring vessel whereby the jet of metal between the pouring vessel and the receiving mold in contact with the air forms a rigid hose through which the remainder of the metal in the pouring vessel can flow without 60 contact with the air.

65 3. A method of protecting a jet of molten magnesium and high-percentage magnesium alloys from oxidation, comprising the step of keeping the point of issue of the metal from the pouring vessel in a substantially 70 fixed position relative to the gate of the receiving mold and adding to the atmosphere surrounding the molten metal a substance capable of forming a coherent film on the 75 molten metal.

4. A method of protecting a jet of molten magnesium and high-percentage magnesium alloys from oxidation, comprising the step of keeping the point of issue of the metal from the pouring vessel in a substantially 70 fixed position relative to the gate of the receiving mold and adding to the atmosphere surrounding the molten metal a substance capable of forming, in co-action with air, a coherent film on the molten metal.

5. A method of protecting a jet of molten magnesium and high-percentage magnesium alloys from oxidation, comprising the step of keeping the point of issue of the metal from the pouring vessel in a substantially 80 fixed position relative to the gate of the receiving mold and adding to the atmosphere surrounding the molten metal sulfur in a finely divided form.

6. A method of protecting a jet of molten magnesium and high-percentage magnesium alloys from oxidation, comprising the step of keeping the point of issue of the metal from the pouring vessel in a substantially 90 fixed position relative to the gate of the receiving mold and spraying sulfur in a finely divided form towards the surface of the molten metal.

In testimony whereof we have hereunto set our hands.

ADOLF BECK.  
WALTHER SCHMIDT.  
GUSTAV SCHREIBER.

95

100

105

110

115

120

125

130